

## UNITED STATES PATENT OFFICE

2,292,308

## LUBRICATING OIL COMPOSITION

Franklin M. Watkins, Chicago, Ill., assignor to  
 Sinclair Refining Company, New York, N. Y., a  
 corporation of Maine

No Drawing. Application October 11, 1940,  
 Serial No. 360,743

18 Claims. (Cl. 252—35)

My invention relates to improvements in compounded petroleum lubricating oils. More particularly, this invention relates to improvements in liquid petroleum lubricants as distinguished from solid or semi-solid petroleum greases. The improved lubricating oil compositions of my invention consist essentially of a petroleum lubricating oil and a metal salt of an alkyl mono-ester of an alkenyl substituted succinic acid, or a mixture of a normal and a basic metal salt of an alkyl mono-ester of an alkenyl substituted succinic acid, in amount, or amounts, insufficient materially to alter the normal liquid character of the petroleum lubricating oil itself. The term "petroleum lubricating oils" is intended to refer herein to lubricating oils of petroleum origin having viscosities upwards of about 50-70 seconds Saybolt Universal at 100° F.

The trend of development in internal combustion engines has imposed increasing burdens upon the oils used and their lubrication, particularly with respect to operating temperatures and pressures. At present, the Diesel type of engine probably represents extreme requirements in both of these respects, but it is not alone in the imposition of severe burdens upon the lubricating oil used. The useful operating life of a lubricating oil in such service is determined in large measure by its thermal stability and by its physical capacity to continue functioning as a lubricant at the high temperatures and high pressures encountered. One measure of thermal stability is resistance to oxidation, and the consequent tendency to form sludge, but in another aspect the effect of thermal instability is determined not only by the extent of oxidation or decomposition but also by the character of the products of such decomposition or oxidation and by the extent and location, within the engine, of deposits of such products.

The improved lubricating oil compositions of my invention have, in addition to the lubricating properties of the petroleum oil of which they are compounded, a high solvent capacity for sludge, of the character formed by oxidation of petroleum lubricating oils and, perhaps of even greater importance, the properties of rendering deposits of sludge and "carbon" within the engine soft and friable rather than hard and coherent and of disintegrating and removing such deposits as an incident of the normal operation of the engine. In this aspect, the lubricating oil compositions of my invention render the engines in which they are used self-cleaning to an important extent.

In the Diesel type of engine, for example, the

high temperatures to which the lubricating oil is subjected, particularly at the top of the stroke, frequently causes deposition of sludge and carbonization in the groove for and behind one or more of the piston rings. Using paraffinic type lubricating oils such difficulties are usually more pronounced with respect to the uppermost ring; using naphthenic type lubricating oils they are usually more pronounced with respect to the lower rings. Consequent sticking of the rings rapidly deprives the pistons and cylinder wall of proper lubrication inducing excessive wear and, frequently, scoring of the cylinder wall. The formation of such "carbon" deposits, hard enough and coherent enough to involve sticking of the rings, is materially retarded, if not avoided, by the use of the improved lubricating oil compositions of my invention. In this aspect the self-cleaning properties of the lubricating oil compositions of my invention, with respect to the engine, make a mere change of oil a substitute, economical with respect both to loss of service time and cost, for the many otherwise necessary cleaning and repair jobs.

25 The class of metal salts of alkyl mono-esters of an alkenyl substituted succinic acid compounded with a petroleum lubricating oil with effective results in accordance with my invention may be represented by the following isometric structural formulae:



or



wherein R is an alkenyl group, R' is an alkyl group, and X is a metal in the form of a normal or basic salt. By "alkenyl" is meant a hydrocarbon group containing a double-bond, such, for example, as the hydrocarbons produced by polymerization of olefins, although other hydrocarbon groups containing a double-bond from other sources may be used. The laurenyl group is an example of such an alkenyl radical, this "laurenyl" group comprising the trimer of iso-butylene obtained by the phosphoric acid polymerization of iso-butylene. The butyl and lauryl groups are examples of an alkyl group although other alkyl groups may be used with advantage. I have found the calcium salts of alkyl mono-esters of alkenyl substituted succinic acid to be particularly effective in accordance with my invention, the calcium being present either as the normal salt or as the basic salt, or a mixture of

the normal and basic salts may be used. However, the corresponding salts of other metals may be used with advantage to produce the improved compounded lubricating oil of the present invention. For example, aluminum, barium, cadmium, chromium, magnesium, nickel, stannous tin, and zinc salts of alkyl mono-esters of alkenyl substituted succinic acid may be used with effective results in accordance with my invention.

The metal salts used in accordance with my invention may be prepared by first reacting maleic anhydride with a suitable olefin at an elevated temperature under suitable pressure. The alkenyl succinic anhydride thus produced may then be converted to the alkyl mono-ester of the alkenyl substituted succinic acid by reacting the anhydride with a metal alcoholate, such as the sodium alcoholate, of an alcohol having the desired alkyl group. A normal metal salt of the resulting mono-sodium salt of the alkyl mono-ester of the alkenyl substituted succinic acid of my invention may be formed by the reaction between the mono-ester mono-sodium salt and a metal salt (such for example as calcium chloride). The basic metal salt may be prepared by liberating the free mono-acid, mono-succinic ester and by reacting this free acid in anhydrous benzene with a substantial excess of metal hydroxide (such for example as calcium hydroxide). It must be understood, however, that the metal salts used in accordance with my invention are not limited to this particular mode of preparation and include such metal salts as are described herein regardless of their source and method of preparation.

The basic calcium salt of the lauryl mono-ester of laurenlyl succinic acid for compounding an example of the improved lubricating oil compositions of my invention can be produced as follows: equimolar parts by weight of dodecene (a trimer of iso-butylene) and maleic anhydride are heated for about 4½ hrs. at 400° F. under a super-atmospheric pressure. The reaction product is placed in a still and the unreacted dodecene and maleic anhydride are distilled off up to a final temperature of 450° F. at 60 mm. pressure. The dodecene and maleic anhydride thus removed by distillation are then reacted together for a second reaction period of about 4 hours at a temperature of about 420-430° F. under super-atmospheric pressure, and the resulting reaction product is again distilled to remove unreacted dodecene and maleic anhydride. The combined yield from these two reactions, totaling upwards of about 50% and obtained as the still residues from the two distillations, has the appearance of a reddish viscous oil and comprises laurenlyl succinic anhydride having a saponification number of 392. One molecular weight each of metallic sodium and lauryl alcohol are then reacted together and are suspended in benzene. One molecular weight of the laurenlyl succinic anhydride is then added to this benzene-sodium-sodium laurylate mixture. The mixture is refluxed for about 3 hours, sodium is washed out of the refluxed mixed with aqueous acid, and the benzene is distilled from this product. The benzene-free product comprises the lauryl mono-ester of laurenlyl succinic acid and has an acid number of about 117.5. The basic calcium salt is then prepared by heating a benzene solution of the lauryl mono-ester of laurenlyl succinic acid with a large excess (about five mols to one) of calcium hydroxide. The mixture is refluxed for about two hours at 80° F. The resulting benzene solution

is filtered to remove unreacted calcium hydroxide, and the benzene is removed by distillation up to a final temperature of 250° F. under a vacuum corresponding to about 4 mm. of mercury. The residue from this distillation comprises the basic calcium salt of the lauryl mono-ester of laurenlyl succinic acid apparently in the form of a mixture of the normal and the basic calcium salts of the lauryl mono-ester of laurenlyl succinic acid. 10 The basic calcium salt thus produced (comprising a mixture of the normal and basic calcium salts) contains about 6.3% calcium by weight with only a trace of sodium.

The preparation of a normal calcium salt of 15 an alkyl mono-ester of an alkenyl substituted succinic acid may be effected by the following method of obtaining, by way of example, the normal calcium salt of the butyl mono-ester of laurenlyl succinic acid. Laurenlyl succinic anhydride is reacted with an equimolar proportion of sodium butylate in boiling benzene solution to form the sodium salt of butyl mono-ester of laurenlyl succinic acid. An aqueous alcohol solution of calcium chloride is then added with vigorous stirring with the resulting formation, by a double decomposition reaction, of the normal calcium salt of the butyl mono-ester of laurenlyl succinic acid. The benzene solution of this normal calcium salt is then washed with water to 25 remove alcohol and inorganic salts (sodium chloride). The washed benzene solution is then filtered and is heated under sub-atmospheric pressure to remove benzene and any alcohol and water remaining in the benzene solution. The resulting normal calcium salt of the butyl mono-ester of laurenlyl succinic acid is a dark colored waxy solid material containing 5.13% calcium. This normal calcium salt may be transformed into the corresponding basic calcium salt by agitating the normal calcium salt with hydrochloric acid and by then adding a large excess (five mols to one) of calcium hydroxide and refluxing this mixture with benzene. Excess calcium hydroxide is removed by filtration and benzene is removed by distillation. The resulting basic calcium salt of the butyl mono-ester of laurenlyl succinic acid is a dark, brittle, resinous product containing about 8% calcium by weight and appears to comprise a mixture of about 55% of the basic calcium salt and about 45% of the normal calcium salt of the butyl mono-ester of laurenlyl succinic acid. 30

In compounding the improved lubricating oil compositions of my invention with Pennsylvania, Gulf Coast or Mid-Continent petroleum lubricating oils, including such oils which have been solvent refined, the metal salt of an alkyl mono-ester of an alkenyl substituted succinic acid, or a mixture of these metal salts, is added to the lubricating oil in amounts ranging from about 40 0.5% up to about 2.5% or 3% by weight on the oil, or even higher. Within this range I have found that amounts of these metal salts corresponding to about 1½% by weight on the oil are particularly effective. The basic calcium salt of the lauryl mono-ester of laurenlyl succinic acid, prepared as described above, is completely soluble to the extent of 1½% by weight in a Gulf Coast oil, a Mid-Continent oil, a Pennsylvania paraffin-base oil, and a Pennsylvania paraffin-base oil which has been twice refined with a mixture of nitrobenzene and sulphuric acid, the latter oil being an example of a high viscosity index aircraft oil. In fact, this basic calcium salt is soluble to the extent of upwards of 17% by weight in a South Texas (Gulf Coast) lubricat-

ing oil and upwards of 8% by weight in a Mid-Continent lubricating oil. The neutral calcium salt of the butyl mono-ester of laurenyl succinic acid and the basic calcium salt of the butyl mono-ester of laurenyl succinic acid, both prepared as described above, are also readily soluble to the extent of at least 1 1/3% by weight in Gulf Coast, Mid-Continent and Pennsylvania lubricating oils but are soluble only to the extent of approximately 1% in a double solvent refined Pennsylvania oil.

As an example of a liquid lubricating oil composition of my invention, a composition consisting essentially of a South Texas pale oil (a Gulf Coast oil), having a viscosity of about 500 seconds at 100° F. Saybolt Universal and boiling 10% up to 700° F. and 90% up to 900° F., approximately, and 1 1/3% by weight on the oil of a basic calcium salt of the lauryl mono-ester of laurenyl succinic acid, produced as described hereinabove, is particularly advantageous. The stability of this lubricating oil composition, as shown by the "Indiana Oxidation Test" described in the S. A. E. Journal 34, 172-173 (1934), is much greater than the stability of this South Texas base oil alone. The Indiana Oxidation Test sludging time with the base oil was 17.0 hours as compared to 26.5 hours for the compounded lubricating oil composition thus representing an increase of about 56% in the sludging time for the compounded oil. In service in a Diesel type engine, this lubricating oil composition left the engine free from sludge or carbon deposits except for a slight discoloration of the piston just above the lower compression rings and a small amount of carbon on the anti-thrust side of the uppermost ring groove of the piston and adequately lubricated the moving parts of the engine. The properties of this particular lubricating oil composition, as compared to those of the lubricating oil alone, as determined in one instance, were as follows:

|                                                     | South Texas oil | South Texas oil+1 1/3% basic calcium salt of lauryl mono-ester of laurenyl succinic acid |
|-----------------------------------------------------|-----------------|------------------------------------------------------------------------------------------|
| Gravity.....° API                                   | 20.0            | 20.2                                                                                     |
| Flash.....° F.                                      | 390             | 385                                                                                      |
| Fire.....do.                                        | 445             | 440                                                                                      |
| Viscosity 100° F., Saybolt Universal seconds.....   | 506             | 524.2                                                                                    |
| Viscosity at 210° F. Saybolt Universal seconds..... | 52.8            | 53.9                                                                                     |
| Viscosity index.....                                | 5.6             | 14.0                                                                                     |
| Pour.....                                           | -10             | -10                                                                                      |
| Carbon residue.....                                 | 0.007           | 0.108                                                                                    |
| Ash.....                                            | 0.0             | 0.210                                                                                    |
| Acid No.....                                        | 0.087           | 0.075                                                                                    |
| Saponification No.....                              | 0.25            | 1.8                                                                                      |

While the lubricating oil composition of the foregoing example embodies specifically a South Texas (Gulf Coast) lubricating oil, other lubricating oil compositions of my invention embodying petroleum lubricating oil from paraffin base crudes, asphaltic base crudes and mixed base crudes are useful. For example, about 1 1/3% by weight of the basic calcium salt of the lauryl mono-ester of laurenyl succinic acid, prepared as described hereinabove, increased the sludging time in the Indiana oxidation test by 61% in the case of a Mid-Continent medium-heavy oil having a viscosity index of 77.9 and by 143% in the case of a Pennsylvania-type lubricating oil having a viscosity index of 102.1. The neutral calcium salt of the butyl mono-ester of laurenyl succinic

acid, prepared as described hereinabove, increased the sludging time, determined by the Indiana oxidation test, by about 10% in the case of a South Texas oil having a viscosity index of 12.4 and by 106% in the case of a Pennsylvania lubricating oil having a viscosity index of 102.5, the neutral calcium salt being incorporated in these oils to the extent of about 1 1/3% by weight on the oil in each instance. The basic calcium salt of the butyl mono-ester of laurenyl succinic acid, prepared as described above, increased the sludging time by 48% in the case of the same South Texas lubricating oil having a viscosity index of 12.4 and by 151% in the case of the same Pennsylvania lubricating oil having a viscosity index of 102.1, the basic calcium salt also being incorporated in these oils to the extent of about 1 1/3% by weight on the oil in each instance.

The metal salts of alkyl mono-esters of an alkenyl substituted succinic acid, being readily soluble in petroleum lubricating oils having high viscosity indices as well as in petroleum lubricating oils having low viscosity indices, are effective anti-sludging compounds of wide applicability to oils obtained from different sources and having either high or low viscosity indices. These metal salts do not materially alter the physical properties of the lubricating oils with which they are compounded, do not cause jelling of the compounded oils, and do not increase the pour point of the base oils with which they are compounded. The compounded lubricating oils of my invention show markedly reduced lacquer and sludge formation in service in Diesel type engines as compared with the un compounded base oils alone. The metal salts further exhibit outstanding sludge stabilizing properties, as shown by the Indiana oxidation test and particularly in the case of lubricating oils obtained from Pennsylvania paraffinic crude oils.

I claim:

1. A liquid lubricating oil composition comprising a petroleum lubricating oil and a metal salt of an alkyl mono-ester of an alkenyl substituted succinic acid, the metal being selected from the group consisting of calcium, aluminum, barium, cadmium, chromium, magnesium, nickel, stannous tin, and zinc.

2. A liquid lubricating oil composition comprising a petroleum lubricating oil and a metal salt of an alkyl mono-ester of laurenyl succinic acid, the metal being selected from the group consisting of calcium, aluminum, barium, cadmium, chromium, magnesium, nickel, stannous tin, and zinc.

3. A liquid lubricating oil composition comprising a petroleum lubricating oil and a calcium salt of an alkyl mono-ester of an alkenyl substituted succinic acid.

4. A liquid lubricating oil composition comprising a petroleum lubricating oil and a calcium salt of an alkyl mono-ester of laurenyl succinic acid.

5. A liquid lubricating oil composition comprising a petroleum lubricating oil and a calcium salt of an alkyl mono-ester of succinic acid, said acid having substituted therein a trimer of isobutylene.

6. A liquid lubricating oil composition comprising a petroleum lubricating oil and a calcium salt of an alkyl mono-ester of the product obtained by reacting maleic anhydride and an olefin at an elevated temperature under pressure.

7. A liquid lubricating oil composition comprising a petroleum lubricating oil and a mixture

of normal and basic calcium salts of the lauryl mono-ester of an alkenyl substituted succinic acid.

8. A liquid lubricating oil composition comprising a petroleum lubricating oil and a calcium salt of the lauryl mono-ester of an alkenyl substituted succinic acid.

9. A liquid lubricating oil composition comprising a petroleum lubricating oil and a basic calcium salt of the lauryl mono-ester of an alkenyl substituted succinic acid.

10. A liquid lubricating oil composition comprising a petroleum lubricating oil and a mixture of normal and basic calcium salts of the butyl mono-ester of an alkenyl substituted succinic acid.

11. A liquid lubricating oil composition comprising a petroleum lubricating oil and a calcium salt of the butyl mono-ester of an alkenyl substituted succinic acid.

12. A liquid lubricating oil composition comprising a petroleum lubricating oil and a basic calcium salt of the butyl mono-ester of an alkenyl substituted succinic acid.

13. A liquid lubricating oil composition com-

prising a petroleum lubricating oil and a mixture of normal and basic calcium salts of the lauryl mono-ester of laurenlyl succinic acid.

14. A liquid lubricating oil composition comprising a petroleum lubricating oil and a calcium salt of the lauryl mono-ester of laurenlyl succinic acid.

15. A liquid lubricating oil composition comprising a petroleum lubricating oil and a basic calcium salt of the lauryl mono-ester of laurenlyl succinic acid.

16. A liquid lubricating oil composition comprising a petroleum lubricating oil and a mixture of normal and basic calcium salts of the butyl mono-ester of laurenlyl succinic acid.

17. A liquid lubricating oil composition comprising a petroleum lubricating oil and a calcium salt of the butyl mono-ester of laurenlyl succinic acid.

20 18. A liquid lubricating oil composition comprising a petroleum lubricating oil and a basic calcium salt of the butyl mono-ester of laurenlyl succinic acid.

FRANKLIN M. WATKINS.